

Patented May 12, 1925.

1,537,518

# UNITED STATES PATENT OFFICE.

JOHN A. WILSON, OF ELIZABETH, NEW JERSEY, ASSIGNOR TO DURATEX CORPORATION, OF NEWARK, NEW JERSEY, A CORPORATION OF NEW JERSEY.

## COATED FABRIC AND METHOD OF MAKING SAME.

No Drawing.

Application filed March 9, 1920. Serial No. 384,571.

To all whom it may concern:

Be it known that I, JOHN A. WILSON, residing at Elizabeth, New Jersey, have invented certain new and useful Improvements in Coated Fabrics and Methods of Making Same, of which I declare the following to be a full, clear, and exact description.

This invention relates to improvement in coated fabrics and the method of making same. It relates more particularly to rubber-coated fabrics, such as may be used for the manufacture of raincoats, slickers, and similar products.

15 The principal object of my invention is to produce a coated fabric having a tough, resilient, and thoroughly waterproof coating which is, at the same time, of light weight and may be produced at a low cost.

20 A further object of my invention is to provide an improved process, or method, for making coated fabrics, by which a light-weight, waterproof, coated fabric may be produced at a low cost.

25 Further objects of my invention will definitely appear from the detailed description to follow.

In general, I carry out the objects of my invention by applying to a suitable fabric base a coating composition made up of a mixture of rubber and a chemically inert, finely divided organic substance, such as comminuted cork or cork flour. This coating composition is applied to the fabric base in any suitable manner and then vulcanized on said base.

I have secured very desirable results by the use of a mixture of sixty (60) pounds of crude rubber and forty (40) pounds comminuted cork or cork flour. To this mixture the desired pigment, cure and accelerator is added, as is well known in the art, and one hundred twenty-five (125) pounds of naphtha are added to the mixture to render it plastic or semi-fluid so that it can be worked and spread.

This mixture is spread upon a suitable fabric base, for instance, napped moleskin, by the use of any suitable spreading or coating means such as are well known in the art. After the coating composition has been spread on the fabric base, the evaporation of the naphtha leaves the coating partly hardened and the coated fabric is then cured, in the manner well known in the art,

vulcanizing the coating on the fabric base.

The addition of the cork does not detract materially from the toughness, elasticity and waterproofing qualities of the rubber and the cork serves as an inert filler which, 60 since it is of a low specific gravity, high resiliency and is not readily permeable to water, gives the body or bulk without a large increase in weight. This enables me to produce a light-weight coated fabric of 65 a quality equal or superior to the heavier rubber-coated fabrics heretofore produced. I have found that desirable results are secured by the use of cork as the filler, but I substitute other inert, organic substances 70 and also secure good results.

I am aware that the particular embodiment of my invention here shown is susceptible of considerable variation without departing from the spirit thereof, and therefore, I 75 desire to claim the same broadly, as well as specifically, as indicated by appended claims.

Having thus described my invention what I claim as new and desire to secure by 80 Letters Patent, is:—

1. A coated fabric comprising a fabric base having applied thereto a mixture of rubber and inert, resilient organic material of low density and not readily permeable to 85 water.

2. A coated fabric comprising a fabric base carrying a coating composed of a mixture of rubber and comminuted cork.

3. A coated fabric comprising a fabric base carrying a coating composed of a mixture of substantially sixty per cent rubber and forty per cent comminuted cork.

4. A coated fabric comprising a fabric base carrying a vulcanized coating composed of a mixture of rubber and inert, resilient material of low density and substantially non-permeable to water.

5. A coated fabric comprising a fabric base carrying a vulcanized coating composed of a mixture of rubber and inert, resilient material of relatively low specific gravity.

6. A coated fabric comprising a fabric base carrying a vulcanized coating composed of a mixture of rubber and comminuted cork.

7. A method of making a coated fabric comprising, mixing crude rubber with a relatively inert material of specific gravity less than one, adding an amount of evap-

- 2
- orale or relatively fugitive substance to render the mixture fluid, applying the same to a fabric base, causing evaporation of said substance, and curing the applied coating.
- 5 8. A method of making a coated fabric comprising, mixing crude rubber with comminuted cork, adding an amount of an evaporable substance to render the mixture fluid, applying the same to a fabric base and thereafter vulcanizing the applied coating.
- 10 9. A method of making a coated fabric which comprises mixing crude rubber with an inert resilient organic material to form a light weight waterproof coating, adding
- 15 a carrier to render said mixture capable of being applied to a fabric base, applying the same to a fabric base and causing an evaporation of said carrier.
10. A method of making a coated fabric comprising, mixing crude rubber with a 20 comminuted light weight flexible material, adding to said mixture a carrier adapted to render the mixture capable of being applied to a fabric base, applying the same to said fabric base, causing an evaporation of said carrier and vulcanizing the said coating on said base.
11. A method of making a coated fabric comprising, applying a coating, containing rubber and cork mixed to render the same 25 capable of being applied to fabric, and vulcanizing the said coating on said fabric.

In testimony whereof, I affix my signature.

JOHN A. WILSON.